

1

3,737,316

**TWO-EQUIVALENT SULFONAMIDO COUPLERS**  
Ilmari Fritiof Salminen and Anthony Loria, Rochester,  
N.Y., assignors to Eastman Kodak Company, Rochester,  
N.Y.

No Drawing. Filed Aug. 31, 1971, Ser. No. 176,684  
Int. Cl. G03c 7/00

U.S. Cl. 96—56.6

28 Claims

**ABSTRACT OF THE DISCLOSURE**

4-sulfonamido-substituted two-equivalent phenol- or  $\alpha$ -naphthol-type cyan dye-forming photographic couplers in color developing compositions, in color photographic silver halide emulsion compositions; elements having such emulsion compositions coated thereon, and processes utilizing such elements.

This invention relates to 4-sulfonamido-substituted two-equivalent phenol- or  $\alpha$ -naphthol-type cyan dye-forming couplers.

Color photographic images are obtained in the photographic art by coupling a silver image development by-product (i.e., oxidized aromatic primary amino developing agents) with a color-forming coupler compound. The subtractive process of color formation is ordinarily employed and the resulting cyan, magenta or yellow image dyes are complementary to the primary colors. Coupler compounds employed to produce cyan photographic dyes, for instance, generally contain phenolic or  $\alpha$ -naphtholic moieties.

Such phenolic or  $\alpha$ -naphtholic couplers usually have various substituent groups on the ring which are capable of affecting various physical characteristics of the compound. Heavy substituent groups, for instance, may act as ballasting groups and tend to decrease solubility in aqueous alkaline processing compositions while increasing non-diffusible characteristics of a coupler in the hydrophilic layers of photo-elements during processing; the corresponding introduction of substituent groups such as halo or alkyl elsewhere on the same ring, however, may adversely or beneficially change the light stability of the image dye produced upon exposure and color development. The presence of an acylamido group on the ring may affect heat stability of some compounds, while the  $D_{max}$  value of a photographic image dye is sometimes increased by substitution of various other groups onto the No. 2 position on the aromatic nucleus. The above-described changes are obviously not uniformly predictable or necessarily beneficial for all color photographic purposes.

In a color photographic system the color-forming coupler may be the unballasted or diffusible type which is conveniently introduced as part of the developing solution, or of the non-diffusible ballasted type which is initially incorporated into or contiguous with a light-sensitive photographic silver halide emulsion layer, both types being made available to react with oxidized color developing agent as a function of silver halide development to obtain a substantially non-diffusible image dye.

Conventional color-forming coupler compounds of the phenolic or  $\alpha$ -naphtholic configuration have an active  $-\text{CH}=\text{}$  group at the No. 4 ring position which reacts with oxidized color developer, as indicated above, to produce an indoaniline dye. Dye-forming color photographic couplers of the above types are known and described as "four-equivalent" couplers, and are characterized in requiring the development of four light-exposed silver halide molecules in order to produce one molecule of dye.

Non-diffusible couplers of the four-equivalent type are

2

exemplified, for instance, in U.S. Pats. 2,895,826, 2,474,293 and 2,908,573. Known diffusible (i.e., unballasted or lightly ballasted) couplers are conveniently exemplified in U.S. Pats. 2,113,329, 2,252,718 and 3,002,836.

5 Two-equivalent dye-forming couplers of the diffusible and non-diffusible types are functionally characterized by requiring the development of only two exposed silver halide molecules during development to obtain one molecule of dye. Such couplers are generally derived from corresponding four-equivalent couplers of either diffusible or non-diffusible types by replacing an available H atom in a coupling position (e.g., No. 4 ring position of a phenol or  $\alpha$ -naphthol ring of a cyan dye-forming coupler) with a nonchromophoric coupling off group such as a fluorine atom, a chlorine atom, an acyloxy group, an aryloxy, an alkoxy, an arylthio, a cycloxy group or a thiocyanato group.

Both two-equivalent and four-equivalent type couplers of the water-soluble (i.e., Fischer type) and non-water-soluble types are utilized for present day color photographic purposes since the combination of characteristics required by modern technology may vary widely.

By way of example, it is important to obtain thinner, more durable photographic elements containing stable 20 couplers which, in turn, produce light- and heat-stable photographic dyes having precise spectral absorption characteristics. The quality of the photographic image, for instance, depends to a large extent upon the relative solubility of certain coupler compounds in high- and/or 25 low-boiling organic solvents as described and utilized, for instance, in Julian, U.S. Pat. 2,949,360, in the light of earlier disclosures in Mannes, U.S. Pat. 2,304,939; Jelley et al., U.S. Pat. 2,322,827; Vittum, U.S. Pat. 2,801,170; and Fierke, U.S. Pat. 2,801,171. The use of minimal 30 amounts of coupler solvent is desirable since the bulk, durability and optical opacity of the resulting photographic element is directly correlated to the amount of solvent employed and retained. This, in turn, affects image definition and resolution properties of the element.

35 Of equal importance is the need for non-diffusible couplers which may be homogeneously incorporated into silver halide emulsions in carefully controlled amounts without adversely affecting viscosity, adhesion, or the unity 40 of any particular emulsion layer during modern high speed multilayer application onto a film backing. Un- 45 desired changes in viscosity of melted gelatin photographic emulsions may be caused by additives such as wetting agents, color components, type of gelatin, etc., and these changes directly affect the coating characteristics of a 50 photographic emulsion.

Including antihalation and gelatin interlayers, up to eight or more separate layers may be applied to a film base to obtain a modern color photographic element 55 [ref. Kirk-Othmer, Vol. 5, pp. 812-845, (1964), "Encyclopedia of Chemical Technology"]. For this reason, any major coupler-induced changes in the adhesion or coating characteristics of a photographic layer are unacceptable. This general problem is recognized, for instance, on page 250 of the text by Zelikman and Levi, entitled "Making and Coating Photographic Emulsions," The Focal Press, (1964), and also in British Pat. 1,193,321.

60 To achieve the above-indicated beneficial characteristics and to avoid corresponding undesirable features for modern color photographic purposes, it is necessary to ascertain which particular group of substituents favor a minimal number of undesirable characteristics while, at the same time, encourage a pre-conceived spectrum of favorable characteristics.

65 It is known, for instance, from U.S. Pat. 2,362,598 of Vittum et al. that some couplers having sulfonamido substituents on the ring tend to form dyes having deficient

heat and light stability. Improvement has been obtained in such cases, however, by attaching the nitrogen atom of the sulfonamido group to the No. 5 or 6 carbon (i.e., non-coupling positions) of the phenolic or naphtholic ring.

In addition, the known difficulty in obtaining non-diffusible type azine dyes from certain ballasted (non-diffusible) couplers is partly resolved in accordance with U.S. Pat. 2,569,906 of Starke by incorporating two ballasted alkyl or aryl sulfonamido groups onto a phenolic or aniline ring, the No. 4 position (coupling position) of the ring being specifically excluded from such substitution.

From U.S. Pat. 2,536,010 of Schmidt et al., it is ascertained that phenolic-type couplers do not readily form azine dye images (i.e., effect ring closure) unless the phenol ring is substituted in the meta position with an alkyl or aryl sulfonamido group.

It is not apparent, from the above teaching, whether certain sulfonamido substituent groups in the No. 4 coupling position will

(1) remain functionally active in a beneficial way, or  
(2) will beneficially affect heat and light stability of the resulting dye obtained from the two-equivalent coupler compound as compared with the corresponding four-equivalent coupler compound.

It is an object of the present invention to obtain a new group of cyan dye-producing coupler compounds, corresponding color photographic emulsions, developer solutions and color photographic elements containing such coupler compounds.

It is a further object to obtain new cyan dye-producing two-equivalent coupler compounds which are easily obtained and which additionally produce dyes having improved light and heat stability as compared with corresponding known four-equivalent couplers.

It is a still further object to achieve the above objects without corresponding loss in image definition or resolution characteristics of a photographic element or material utilizing the new coupler, and without effecting undesirable viscosity changes in a photographic emulsion containing such couplers prior to or during application onto a film base or emulsion support.

The above objects are accomplished, for instance, by utilizing a 4-sulfonamido-substituted phenol- or a 4-sulfonamido-substituted  $\alpha$ -naphthol-two-equivalent cyan dye-forming photographic coupler in which the amido moiety of the 4-sulfonamido substituent is attached to the No. 4 carbon atom of the phenol or  $\alpha$ -naphthol ring. Such compounds can be used in a photographic color processing composition, as well as in photographic silver halide emulsions. This unique class of coupler compounds is conveniently described in the general formula



wherein COUP is the residue of a cyan dye-forming coupler moiety of the phenolic or  $\alpha$ -naphtholic type. Such chemical groups include recognized classes of cyan-dye forming four-equivalent couplers which are normally unsubstituted in the No. 4 position;

wherein  $\text{R}_1-\text{SO}_2-\text{NH}-$  preferably represents a non-chromophoric radical attached onto the No. 4 carbon of the phenolic- or  $\alpha$ -naphtholic-ring of COUP-; and

$\text{R}_1$  is an alkyl or an aryl group, inclusive of straight or branched alkyls of 1-20 carbon atoms, exemplified by methyl, isopropyl, octadecyl and eicosyl, also an aryl group such as a phenyl or a naphthyl radical and inclusive of phenyl, naphthyl, and substituted phenyl or substituted naphthyl having at least one ring substituent such as an alkyl or alkoxy having alkyl moieties of 1-20 carbon atoms, also a ring substituent such as a nitro, a carboxy, a halo (e.g., chloro) or an alkyl-substituted carbonyl group such as propyl carboxy.

Diffusible and non-diffusible couplers utilized within

the scope of the present invention can also be conveniently represented by the general formulae:



or



in which (PHOL) and (NAOL) are defined respectively as a cyan dye-forming coupler moiety of the phenolic- or the  $\alpha$ -naphtholic-type, both having at least two ring substituent groups on the phenolic or  $\alpha$ -naphtholic ring in addition to a hydroxyl radical; the

$\text{R}_1-\text{SO}_2-\text{NH}$ -group is defined as above and conveniently described as a wholly displaceable group upon reaction with oxidized color developer during color development,

the  $\text{R}_1$  moiety alone or in combination with any other part of the No. 4 substituent group being a non-chromophoric group which is further defined as being neither a photographic dye nor a diffusible dye precursor of the type capable of a hypsochromic or bathochromic shift when subjected to a different environment such as a change in pH. Compounds utilizing preformed dyes or dye precursors of the type here excluded are disclosed, for instance, in a copending application by Fleckenstein, U.S. application Ser. No. 282,796 entitled "Novel Sulfonamido Phenols," and in U.S. Pat. 2,756,142; the  $\text{R}_3$  group is also more precisely described as a No. 2 phenolic-ring substituent defined as a hydrogen atom, an alkyl group having up to 30 carbon atoms and preferably alkyl of 1-20 carbon atoms such as methyl, isopropyl, pentadecyl, and eicosyl, an alkoxy group having up to 30 carbon atoms, preferably alkoxy of 1-20 carbon atoms such as methoxy, isopropoxy, pentadecyloxy and eicosyloxy, or a substituent group of the formulae:



or



wherein  $\text{A}$  is an alkyl group including an unsubstituted alkyl having up to 30 carbon atoms and preferably 1-20 carbon atoms, also including a substituted alkyl such as halo alkyl or polyhaloalkyl such as a fluoroalkyl or an aryloxy alkylene group wherein the alkylene moiety preferably contains up to about 15 carbon atoms and the aryloxy moiety, inclusive of a phenoxy or a naphthoxy group, can be additionally substituted by one or more of an alkyl, or alkoxy or a halo group, the alkyl or alkoxy moieties of such additional substituents can contain up to 30 carbon atoms and are exemplified by methyl, propyl, dodecyl, pentadecyl, eicosyl, methoxy and eicosyloxy;  $\text{Ar}$  is defined as an aryl group consisting of a phenyl or a naphthyl group having one or more of an alkyl, an alkoxy and a halo substituent group thereon, the alkyl moieties of said alkyl or alkoxy containing up to 30 carbon atoms and preferably 1-20 carbon atoms;  $\text{R}_7$  is a No. 2-naphtholic ring substituent defined as an alkyl group having up to 30 carbon atoms and preferably about 1-20 carbon atoms or a substituent group of the formulae:



or



wherein  $\text{A}$ ,  $\text{Ar}$  and  $\text{R}_1$  are defined as above.

Corresponding diffusible cyan dye-forming couplers within the present invention are conveniently represented by Formulae 2 and 3 as described above, wherein  $\text{R}_3$  and  $\text{R}_7$  are defined as a hydrogen atom, an alkyl group having up to about 14 carbon atoms or an alkoxy group having up to about 14 carbon atoms such as methyl, dodecyl, methoxy, dodecyloxy, etc., the alkyl and alkoxy groups preferably having a lower alkyl moiety of 1-8 carbon atoms.  $\text{R}_3$  and  $\text{R}_7$  are also respectively defined in diffusible-type couplers as radicals of Formula 4 or 6 above,

wherein A is an alkyl group having up to about 14 carbon atoms and preferably lower alkyl of 1-8 carbons, such groups being exemplified, for instance, by methyl, isopropyl or dodecyl. Diffusible type couplers also preferably have either hydrogen, a halo radical, or lower alkyl group having up to about 8 carbon atoms, or lower alkoxy group having up to about 8 carbon atoms as substituents on the remaining available ring carbon atoms in the phenol or naphthol coupler moiety.

The non-diffusible couplers (i.e., those substantially non-migratory couplers remaining within the light-sensitive silver halide emulsion) essentially constitute the residue of the compounds within the scope of Formulae 1-3 (supra); in particular, those in which R<sub>3</sub> and R<sub>7</sub> are, respectively, No. 2-phenolic or No. 2- $\alpha$ -naphtholic ring substituents defined as an alkyl group having at least about 15 carbon atoms, preferably 15-30 carbons, or defined, respectively, as substituent groups of Formulae 4-5 or 6-7 (supra) in which A is an unsubstituted alkyl group containing at least about 15 carbon atoms and preferably 15-30 carbon atoms, or a substituted alkyl such as an aryloxy alkylene group wherein the alkylene moiety contains up to about 15 carbon atoms, preferably 1-10, and the aryloxy moiety is inclusive of a phenoxy or a naphthoxy group and may be additionally substituted by one or more of an alkyl, an alkoxy, or a halo group, the alkyl or alkoxy moieties of the additional substituents preferably containing about 1-20 carbon atoms; and in which Ar is defined as a phenyl or naphthyl group including those having one or more of an alkyl, an alkoxy and a halo substituent thereon, the alkyl moieties of the alkyl or alkoxy containing at least about 15 carbon atoms.

Two-equivalent photographic coupler compounds of both types within the scope of the present invention also include those represented by the formulae



wherein R<sub>1</sub>, R<sub>3</sub>, R<sub>7</sub>, A, and Ar are defined as above; R<sub>2</sub> is defined as a hydrogen atom, a halo radical such as chloro or fluoro, an alkyl group, including alkyl of 1-20 carbon atoms such as methyl, isopropyl, octyl, octadecyl, eicosyl, and chloromethyl and as an alkoxy group having an alkyl moiety of 1-20 carbon atoms, exemplified by methoxy or eicosyloxy, hydrogen, lower alkyl and lower alkoxy being preferred substituents; R<sub>4</sub> is defined as a hydrogen atom, a halo radical such as chloro or fluoro; an alkyl group preferably lower alkyl of 1-8 carbons such as methyl, isopropyl or octyl, and an alkoxy group, preferably lower alkoxy of 1-8 carbons such as octyloxy; R<sub>5</sub> in

Formula 9 is defined as in R<sub>4</sub>, and in Formula 8 additionally includes a radical of the formula



in which Y is an acyl group including

5 (1) An alkyl carbamyl group such as a substituted or unsubstituted alkanoic acid group having 1-20 carbon atoms including methylcarbonyl, a lauroyl group, an aryloxy alkyl carbonyl such as an alkyl- or dialkylphenoxyalkylcarbonyl and an arylcarbamylalkylcarbonyl such as dimethylcarboxyphenylcarbamylalkylcarbonyl;

10 (2) An arylcarbonyl group such as a phenyl, an alkylphenylhalosulfonylphenyl and corresponding naphthylcarbonyl groups or (3) a heterocyclic carbonyl having 5-6 members in the ring nucleus and exemplified by a furyl group; and R<sub>6</sub> and R<sub>8</sub> are individually defined as a hydrogen atom or an alkyl preferably lower alkyl inclusive of 1-8 carbon atoms such as a methyl or octyl substituent.

15 Substituted sulfonamido couplers included within the present invention are conveniently obtained, for instance, by reacting a corresponding phenol or  $\alpha$ -naphthol 4-amine with the desired aryl sulfonyl halide. The reaction is demonstrated by the equation



wherein X is a halo radical such as chloro, while



30 is a 4-amino substituted four-equivalent cyan dye-producing coupler of the above-defined type, and R<sub>1</sub> is also defined as above.

35 A further reaction mechanism useful for obtaining compounds such as Couplers XXIX-XLI (infra) involves reacting a 2-nitro-4-aminophenol, with benzyl sulfonyl chloride, reducing the 2-nitro group to obtain the amine and then further reacting the intermediate with a suitable alkyl-, aryl-, or heterocyclic-carbonyl chloride, followed by nitration of the number 5 position, reduction of the nitro group, and then reaction of the resulting amine with benzoyl chloride to obtain the desired product.

40 45 Suitable reaction mechanisms for obtaining the above COUP—NH<sub>2</sub>—(PHOL)—NH<sub>2</sub> or —(NAOL)—NH<sub>2</sub> reactant are well known in the art as evident, for instance, from the Fieser text entitled "Advanced Organic Chemistry," pages 620-627, 5th edition (1961), and from the reactions described in producing corresponding four-equivalent and 4-chloro-substituted two-equivalent cyan dye-forming couplers in U.S. Pats. 2,772,162 of Salminen et al. and U.S. Pat. 2,908,573 of Bush et al.

50 55 The following couplers are listed to illustrate the variety of compounds falling within the scope of the invention, it being noted that both diffusible (i.e., introduced during processing of exposed film) and non-diffusible-type couplers are included:

| Coupler                                                                                  | M.P. (°C.) |
|------------------------------------------------------------------------------------------|------------|
| I.   | 154-157    |
| II.  | 187-190    |

| Coupler                                                                                          | M.P. (° C.) |
|--------------------------------------------------------------------------------------------------|-------------|
| III.....<br>    | 195-197     |
| IV.....<br>     | 196-202     |
| V.....<br>      | 199-203     |
| VI.....<br>    | 129-134     |
| VII.....<br>  | 192-200     |
| VIII.....<br> | 200-204     |
| IX.....<br>   | 186-200     |
| X.....<br>    | 133-135     |

| Coupler       | M.P. ° (C.) |
|---------------|-------------|
| XI.....<br>   | 156         |
| XII.....<br>  | 129-131     |
| XIII.....<br> | 202-204     |
| XIV.....<br>  | 186-188     |
| XV.....<br>   | 158-160     |
| XVI.....<br>  | -----       |

Additional couplers within the scope of the present invention include, for instance:

- XVII..... 2-N-dodecylcarbamyl-4-phenylsulfonamido-naphthol.  
 XVIII..... 2-N-octadecylcarbamyl-4-(p-methylphenylsulfonamido)naphthol.  
 XIX..... 2-N-hexadecylcarbamyl-4-(p-octylphenylsulfonamido)naphthol.  
 XX..... 2-N-octadecylcarbamyl-4-(octadecylsulfonamido)naphthol.  
 XXI..... 2-N-octadecylcarbamyl-4-(methylsulfonamido)naphthol.  
 XXII..... 2-(octadecylcarbonamido)-4-(phenylsulfonamido)phenol.  
 XXIII..... 2-(hexadecylcarbonamido)-4-(p-carboxyphenylsulfonamido)phenol; and  
 XXIV..... 2-(dodecylcarbonamido)-4-(p-octylphenylsulfonamido)phenol; also  
 XXV..... 2-pentyl-6-methyl-4-(phenylsulfonamido)phenol.  
 XXVI..... 2-octyloxy-4-(phenylsulfonamido)phenol.  
 XXVII..... 2-octyl-5-methyl-4-(octylsulfonamido)phenol; and  
 XXVIII..... 4-(octadecylsulfonamido)phenol.  
 XXIX..... 2-chloro-3-methyl-4-phenylsulfonamido-6-[ $\alpha$ -(3-n-pentadecylphenoxy)acetamido]phenol.  
 XXX..... 2-acetamido-4-phenylsulfonamido-5-[ $\alpha$ -(2,4-di-tert-amyloxy)acetamido]phenol.  
 XXXI..... 2-[ $\gamma$ -(2,4-di-tert-amyloxy)butyramido]-4-phenylsulfonamido-5-benzamidophenol.  
 XXXII..... 2,5-di-acetamido-4-phenylsulfonamidophenol.  
 XXXIII..... 2,5-di-lauroylamido-4-phenylsulfonamidophenol.  
 XXXIV..... 2-lauroylamido-4-phenylsulfonamido-5-furoylamido-phenol.  
 XXXV..... 2-[ $\gamma$ -(2,4-di-tert-amyloxy)butyramido]-4-phenylsulfonamido-5-[ $\beta$ -(3,5-dicarbomethoxyphenylcarbamyl)valeramido]phenol.

- XXXVI..... 2-[ $\gamma$ -(2,4-di-tert-amyloxy)butyramido]-4-phenylsulfonamido-5-p-tert-amylobenzamidophenol.  
 XXXVII..... 2,5-bis[ $\alpha$ -( $\chi$ -chloro-2,4-di-tert-amyloxy)acetamido]-4-phenylsulfonamido-5-(3-chlorosulfonylbenzamido)-2,4-phenylsulfonamido-5-(3-chlorosulfonylbenzamido)-2-steramidophenol.  
 XXXIX..... 2-( $\alpha$ -heptafluorobutyramido)-4-octadecylsulfonamido-5-[ $\alpha$ -(2,4-di-tert-amyloxy)hexamidophenol.  
 XL..... 2-( $\alpha$ -heptafluorobutyramido)-4-(p-methylphenylsulfonamido)-5-[ $\alpha$ -(2,4-di-tert-amyloxy)hexamidophenol.  
 XLI..... 2-[N-(2,4-di-tert-amyloxy)butylcarbamyl]-4-(m-nitrophenylsulfonamido)-naphthol.

The above compounds include both diffusible and non-diffusible two-equivalent type coupler compounds; couplers I-XIV and XXV-XXVIII, for example, generally represent the diffusible type and XV-XXIV, the non-diffusible type.

Other types of 4-sulfonamido-substituted phenols and naphthol compounds are described in the concurrently filed and pending application of Fleckenstein and Figueras, U.S. Application Ser. No. 176,752, now abandoned and continued in part in Ser. No. 282,795 filed Aug. 22, 1972, entitled "Diffusion Transfer Systems" and Fleckenstein, U.S. Application Ser. No. 176,751, now abandoned and continued in part in Ser. No. 282,796

filed Aug. 22, 1972, entitled "Novel Sulfonamido Phenols," wherein the groups corresponding to R<sub>1</sub> of Formula 1 (*supra*) are a pre-formed diffusible dye or a dye precursor such as a leuco dye or a "shifted" dye which shifts hypsochromically or bathochromically when exposed to a different environment such as a change in pH.

The ballasted non-diffusible type cyan couplers of the present invention are usefully incorporated into light-sensitive photographic silver halide emulsion layers and applied onto an emulsion support or film base in a single- or multi-layer color photographic material by known methods (example: the solvent and Fisher fat-tail methods) as described, for instance, in Mannes et al. in U.S. 2,304,939-40 and Jelley et al. in U.S. Pat. 2,322,027, in which high-boiling organic solvents are used to dissolve the coupler. Further useful procedures are described, for instance, in Vittum et al. U.S. Pat. 2,801,170; Fierke et al. U.S. Pat. 2,801,171 (July 1957); and Julian U.S. Pat. 2,479,360 (August 1960), whereby low-boiling or water-soluble organic solvents are used with or in place of a high-boiling solvent. In the case of multi-layer photographic materials or elements, the non-diffusible coupler compounds are generally incorporated into the red-sensitive silver halide emulsion layer and preferably utilize minimal amounts of high-boiling solvents.

Generally speaking, a useful coupler concentration will vary from about 25-200 mg./ft.<sup>2</sup> of coated material, a range of 30-50 mg./ft.<sup>2</sup> being generally satisfactory for use in photographic paper, with overlapping and higher concentrations found useful in color photographic films.

A variety of color coupler-containing photographic materials and elements are obtainable utilizing the above family of cyan dye-producing couplers. Generally speaking, however, such photographic materials and elements will comprise the following main components:

(A) A support layer such as cellulose nitrate film, cellulose acetate film, polyvinylacetal film, polystyrene film, poly(ethylene terephthalate) film, polyethylene film, polypropylene film and related films of resinous materials as well as paper, polyethylene coated paper, glass, and others. The terms include paper or other flexible fibrous material which can be partially acetylated or coated with baryta or some other hydrophobic film or surface which repels and does not absorb or adsorb water. A support layer having a hydrophobic surface can also include hydrophobic resin layers which have been subject to a corona treatment as described, for instance, in British Pats. 971,058, 1,060,526 and U.S. Pats. 2,864,755 and 2,864,756 to improve adhesion of hydrophilic colloid layers coated over them. Such resin layers or films may be either self-supporting or may be coated over another support layer. Specific supports having useful hydrophobic surfaces include polyethylene terephthalate films electron-bombarded to have a contact angle less than 45° (U.S. Pat. 3,220,842), a corona-treated surface comprising a chromium halide (U.S. Pat. 3,117,865), or corona-treated hardened gelatin coated papers (Belgian Pat. 671,661), etc. The support layer may also contain various functional additives such as titanium dioxide, zinc oxide, and silica as suggested in U.S. Pats. 2,992,101 and 2,701,245, and anti-static agents as described, for instance, in U.S. Pat. 3,253,922;

(B) An antihalation layer such as a dye-containing gelatin, starch, etc., as described, for instance, in Glafkides "Photographic Chemistry," volume 1, pages 470-471, Arrowsmith Ltd. 1958;

(C) One or more, preferably three light-sensitive and differently-sensitized color coupler-containing silver halide emulsion layers coated onto the support, optionally with one or more gelatin spacer layers between. The support is conveniently coated in succession with a red-sensitive layer containing one or more of the above-defined class of cyan-dye-producing coupler, a green-sensitive layer and a blue-sensitive layer, either with or without a Carey-Leit filter layer between the blue- and green-sensitive

layers. The three differently color-sensitized layers can also be arranged in any other order over one another that is desirable, with the exception that a Carey-Lea filter layer cannot be placed over a blue-sensitive layer.

5 The light-sensitive silver halide emulsions can include coarse, regular, or fine grain silver halide crystals or mixtures thereof such as silver chloride, silver bromide, silver bromoiodide, silver chlorobromide, silver chloro-iodide, silver chlorobromoiodide and mixtures thereof; 10 such emulsions are described, for instance, in "The Photographic Journal," volume LXXIX, May 1939, pages 330-338; "Journal of Photographic Science," volume 12, No. 5, Sept./Oct. 1964, pages 242-251, and also in U.S. Pats. 2,184,013, 2,456,953, 2,541,472, 2,563,785, 15 3,367,778 and 3,501,307. In addition to the cyan-dye-forming couplers of the present invention such emulsions used in green- and blue-sensitive layers can include two- and four-equivalent magenta- and yellow-dye-producing couplers of the type described, for instance, in U.S. Pats. 2,453,661, 2,449,966, 2,521,908, 2,908,573, 3,311,476, 20 3,476,563, 3,152,896 and 3,062,653.

Ballasted two-equivalent couplers of the present invention are usefully incorporated within gelatin, colloidal albumin, cellulose derivatives or synthetic resins, as described in U.S. Pat. 2,286,215 or 2,327,808, water-soluble ethanol amine cellulose acetates as described in U.S. Pat. 2,322,085, also suitable polyacrylamides having a combined acrylamide content of 30-60% and a specific viscosity of .25-1.5 on an imidized polycrylamide of similar acrylamide content and viscosity such as described in U.S. Pat. 2,541,474, in Zeil as described in U.S. Pat. 2,563,791, into a vinyl alcohol polymer containing urethane carboxylic acid groups of the type described in U.S. Pat. 2,768,154, or one containing cyano-acetyl groups, 30 exemplified by vinyl alcohol-vinyl cyanoacetate copolymers as described in U.S. Pat. 2,808,331, a polymeric material from a protein polymerisate or a saturated acylated protein with a monomer having a vinyl group described in U.S. Pat. 2,852,382.

40 (D) One or more gelatin spacer layers between the light-sensitive emulsion layers or the emulsion layers and Carey-Lea filter layer as above described; and

(E) A protective water-permeable overcoat layer, such as gelatin, poly-N-vinyl lactam, gum arabic, hydrophilic 45 copolymer of N-acrylamidoalkyl betain (ref. U.S. Pat. 2,833,650), cellulose ethers and esters, alkali soluble polyvinyl phthalate (ref. U.S. Pat. 2,798,004); also water-soluble polymers having varying degrees of solubility, such as polyvinyl alcohol (optimally with surfactant), 50 polyvinyl pyrrolidone polyalkylene oxides, polyvinyl alcohol and its derivatives such as partial esters, ethers and acetals exemplified by hydrolyzed polyvinylacetate, polyvinyl acetaldehyde acetal, polyvinyl butyraldehyde acetal, polyvinyl sodium o-sulfonylbenzaldehyde acetal, polyvinyl disodium 2,4-disulfonylbenzaldehyde acetal; and water-soluble copolymers and interpolymers exemplified by copoly(methyl vinyl ether/maleic anhydride), copoly(acrylic acid/methacrylic acid ethyl ester-maleic anhydride) and copoly(maleic anhydride/acrylic acid/vinyl acetate). 55 The overcoat may conveniently contain aldehyde scavenger such as described, for instance, in U.S. Pats. 3,236-652, 3,287,135, 3,220,839, 2,403,927, and British Pat. 623,448, and other ingredients such as buffering agents (e.g., an acidic or basic material), and ultra-violet light absorbers such as 2,2'-di-hydroxy-4,4'-dimethoxybenzophenone, 4,4'-dimethoxybenzophenone, 4,4'-diazidostilbene-2,2'-disulfonic acid sodium salt, and sodium-( $\alpha$ -phenylhydrazone).

In addition, photographic materials and elements utilizing the present cyan-dye-forming couplers can usefully contain brighteners such as stilbenes, triazines, oxazoles and coumarins as described, for instance, in German Pats. 972,067, 115,024, and in U.S. Pat. 2,933,390; they may also contain spectral sensitizing dyes to impart additional sensitivity to light-sensitive silver halide emulsion layers.

Suitable light-sensitive emulsions for purposes of the present invention can also contain speed-increasing compounds of the quaternary ammonium and polyethylene glycol type as found, for instance, in U.S. Pats. 2,271,623, 2,288,226, 2,334,864 and 2,708,162.

Unballasted or lightly ballasted diffusible two-equivalent couplers within the present invention are usefully introduced into a photographic element during processing by dissolving or otherwise incorporating them into an aqueous alkaline aromatic primary amino color developing solution of a type exemplified by the general formulation

|                                      | G./L. |
|--------------------------------------|-------|
| Development accelerator              | 0-50  |
| Color developing agent               | 2-100 |
| Alkali metal bromide                 | 0-100 |
| Antifoggant                          | 0-1.0 |
| Alkali metal iodide                  | 0-1.0 |
| Alkali metal chloride                | 0-25  |
| Soluble diffusible competing coupler | 0-500 |
| Buffer                               | 0-100 |
| Silver halide solvent                | 0-50  |
| Antioxidant                          | 0-50  |
| pH range, 8.0 to 14.0.               |       |

wherein the pH is conveniently adjusted with an alkali metal or ammonium hydroxide.

Development accelerators for use in the above-type formulation include, for instance:

benzyl alcohol  
p-cresol  
phenyl ethyl alcohol  
p-n-amyl phenol  
n-octyl alcohol and  
p-sec.-butyl phenol

The color developing agents found useful in the present invention are customarily of the p-phenylene-diamine type and include:

p-amino-N,N-diethylaniline HCl  
4-amino-3-methyl-N,N-diethylaniline HCl  
4-amino-N-ethyl-N-β-hydroxyethylaniline H<sub>2</sub>SO<sub>4</sub>  
4-amino-N-butyl-N-ω-sulfonybutylaniline  
4-amino-3-methyl-N-ethyl-N-β-hydroxyethylaniline H<sub>2</sub>SO<sub>4</sub>  
4-amino-3-methyl-N-ethyl-N-β-(methane sulfonamido)ethylaniline 3/2 H<sub>2</sub>SO<sub>4</sub>—H<sub>2</sub>O  
4-amino-3-β-(methanesulfonamido)ethyl-N,N-diethylaniline HCl  
4-amino-3-methoxy-N-ethyl-N-β-hydroxyethyl-aniline 2HCl, and  
N,N-diethyl-3-(2-hydroxyethyl)-p-phenylenediamine 2HCl, while

useful antifoggant components are demonstrated, for instance, by

benzotriazole  
5-nitrobenzimidazol nitrate  
5-nitroindazole  
1-phenyl-5-mercaptopetetrazole  
5-methylbenzotriazole, and  
N-methylbenzothiazolium-p-toluene sulfonate, etc.

Useful buffers in color developing formulations can include alkali metal salts such as:

K<sub>3</sub>PO<sub>4</sub>, K<sub>2</sub>HPO<sub>4</sub>, KH<sub>2</sub>PO<sub>4</sub>, Na<sub>2</sub>CO<sub>3</sub>

an alkali metal salt of boric acid, etc., or organic buffers, such as described in Bard et al., U.S. Pat. 3,305,364, etc.

Useful silver halide solvent for the above purpose includes:

Na<sub>2</sub>S<sub>2</sub>O<sub>3</sub>  
NaCNS  
NH<sub>4</sub>OH  
ethylenediamine

dithiooctanediol  
thiourea  
isopropylamine, and  
n-butylamine, etc.; and  
5 useful antioxidants include:  
hydroxylamine sulfate  
diethylhydroxylamine  
sodium sulfite  
dextrose  
10 p-hydroxyphenyl glycine  
ascorbic acid  
oxytetroanic acids and  
dihydroxyacetone; while  
suitable optional soluble competing couplers are exemplified, for instance, by  
α-pivaloylacet-4-sulfoanilide  
α-pivaloylacet-2-sulfoanilide  
α-pivaloylacet-2,4-dicarboxyanilide  
3-amino-1-(4-sulfophenyl)-5-pyrazolone  
3-(4-sulfoanilino)-1-(chlorophenyl)-5-pyrazolone  
3-amino-1-(4-sulfophenyl)-4-thiocyanato-5-pyrazolone  
1-amino-8-naphthol-3,6-disulfonic acid  
2-amino-5-naphthol-7-sulfonic acid  
1,8-dihydroxynaphthalene-3,6-disulfonic acid  
2,6-dihydroxyisonicotinic acid  
3,5-dihydroxybenzoic acid  
methyl 2,6-dihydroxyisonicotinate  
α-(4-sulfonylbenzoyl)-α-chloroacetanilide  
30 α-(4-carboxybenzoyl)-α-chloro-ω-carboxyacetanilide, and  
α-(4-hydroxybenzoyl)-α-chloro-ω-sulfoacetanilide  
additional competing couplers of this type are further described in U.S. Patent Application S.N. 52,721, now U.S. Patent 3,647,452, of Hendess et al. filed on July 6, 1970.  
35 This invention is further described, although not limited, by the following examples:

#### EXAMPLE I—COUPLER I

A mixture of 17.37 gm. (.1 mol) 4-amino-2,6-dimethylphenol hydrochloride and 150 ml. pyridine are cooled in an ice bath and 19.43 gm. (.11 mol) of benzenesulfonyl chloride added, with stirring, under a nitrogen atmosphere for 2.5 hours. The mixture was thereafter poured onto ice and concentrated HCl and the resulting gummy product, separated and recrystallized from an ethanol-water mixture and identified as 2,6-dimethyl-4-benzene sulfonamido phenol (M.P. 154-157° C.).

#### EXAMPLE II—COUPLER VI

A mixture of .1 mol 4-amino-2,6-dimethyl phenol hydrochloride and 150 ml. pyridine are cooled and slowly reacted with about .11 mol of methylsulfonyl chloride, with stirring, under a nitrogen atmosphere as in Example 1, and the resulting product recovered and recrystallized to obtain a crystalline material identified as 2,6-dimethyl-4-methylsulfonylphenol (M.P. 129-134° C.).

#### EXAMPLE III—COUPLER XV

To 9.8 gm. of 4-amino-2-[α-(2,4-di-tert, amylphenoxy)butyramido]-α-naphthol, obtained in accordance with the process described in Example 1 of U.S. Pat. 2,474,293 is added 100 ml. dry pyridine and then admixed with 3.8 gm. of p-toluenesulfonylchloride, with stirring at room temperature for 2 hours, and heated in a steam bath for ½ hour. The resulting mixture is then poured into 1 liter of water and the oil product separated and crystallized from alcohol (M.P. 158°-160° C.).

Calculated (percent): C, 70.7; H, 7.5; S, 5.0; N, 4.4. Found (percent): C, 70.7; H, 7.5; S, 5.1; N, 4.5.

#### EXAMPLE IV—COUPLER XXIX

70 A mixture of .1 mole of 3-n-pentadecyl phenol, .11 mole of potassium hydroxide pellets, and 150 ml. of xylene is stirred and boiled until 75 ml. of xylene is collected. To the remainder, is added .1 mole of sodium chloroacetate and refluxed for three hours; the product is then cooled

and audified and the crystallized intermediate recovered and reacted with excess thionyl chloride at 50°-56° C. for four hours and the excess thionyl chloride removed under vacuum; .01 mole of the  $\alpha$ -(3-pentadecylphenoxy) acetyl is then reacted in the presence of .03 mole anhydrous sodium acetate in 90% acetic acid with .01 mole of 2-chloro-3-methyl-4-amino-6-nitrophenol hydrochloride obtained from 2-chloro-3-methylphenol by coupling with a diazonium salt, followed by reduction to obtain the  $\alpha$ -amino derivative, and then nitration to the  $\alpha$ -position and reduction; the reaction product of 2-chloro-3-methyl-4-amino-6-nitrophenol and the above-described octyl chloride recovered and identified as Coupler XXIX.

#### EXAMPLE V—COUPLER XXXVIII

To a solution of .1 mole of 5-amino 2-stearamido phenol in 60 volumes dioxane is added .11 mole 3-chlorosulfonylbenzoyl chloride in 15 volumes of dioxane at 25° C.; an aqueous slurry of the product is then filtered, crystallized from ethyl acetate, then nitrated and reduced to the 4-amine, and thereafter reacted with .11 mole of benzylsulfonyl chloride to obtain the corresponding 4-phenyl sulfonylamido derivative identified as Coupler XXXVIII.

#### EXAMPLE VI—COUPLER XXXII

By utilizing .1 mole of 5-amino-2-acetamidophenol and .11 mole of acetyl chloride in place of the 5-amino-2-stearamidophenol and 3-chlorosulfonyl benzoyl chloride in the process of Example V, there is obtained a compound identified as Coupler XXXII.

#### EXAMPLE VII—COUPLER XXXIII

By utilizing .1 mole of 5-amino-2-lauroylamidophenol in place of 5-amino-2-stearamidophenol and .11 mole of laurylsulfonylchloride in place of benzylsulfonyl chloride in the process of Example V, there is obtained a compound identified as Coupler XXXIII.

#### EXAMPLE VIII—COUPLER XXXIV

By utilizing .1 mole of 5-amino-2-lauroylamidophenol in place of 5-amino-2-stearamidophenol and .11 mole of furoyl chloride in place of benzoylsulfonyl chloride in the process of Example V, there is obtained a compound identified as Coupler XXXIV.

#### EXAMPLE IX

Three coupler-free single-layer test strips are prepared by coating cellulose acetate support with light-sensitive gelatin-silver bromoiodide emulsion; the test strips are exposed to a light source through a 0-3.0 D step wedge, and developed to obtain a silver image which is then fixed and treated with  $K_3Fe(CN)_6$  and KBr in the usual manner; the strip is then color developed by introducing the strip into a solution containing 5.15 mol/l. of Coupler I,  $1.5 \times 10^{-2}$  mol/l. of 4-amino-3-methyl-N,N-dimethyl-aniline developer, .65 gm./l. of  $Na_2SO_3$  and 1 gm./l. of KBr buffered to pH 12 with a phosphate buffer. The developed strips are then fixed, bleached, and fixed to obtain a cyan dye image having a  $\tau$  max. of 609 and a  $D_{max}$  of 2.45. Upon testing the developed strips for light and heat fading, values of .09 and .02 respectively, are obtained.

#### EXAMPLE X

(A) Three film test strips are prepared by coating cellulose acetate film base with a single layer of light-sensitive bromoiodide test emulsion, containing gelatin (450 mg./ft.<sup>2</sup>), silver (126 mg./ft.<sup>2</sup>), and a coupler of the formula



(80 mg./ft.<sup>2</sup>) dissolved in dibutyl phthalate (40 mg./ft.<sup>2</sup>) and dispersed into the gelatin. The coated strips are then exposed to a light source through a step wedge and color developed in the usual manner using the following color developer composition:

|    |                                                              |    |      |
|----|--------------------------------------------------------------|----|------|
| 5  | $H_2O$                                                       | ml | 800  |
|    | Sodium hexametaphosphate                                     | g  | 0.5  |
|    | $Na_2SO_3$                                                   | g  | 2.0  |
| 10 | 4 - amino - 3 - methyl - N,N - diethyl aniline hydrochloride | g  | 2.0  |
|    | $Na_2CO_3$ , $H_2O$                                          | g  | 20.0 |
|    | 50% $NaBr$ solution                                          | ml | 3.46 |
|    | $H_2O$ to 1 liter (pH 10.86).                                |    |      |

15 The developed strips are then tested for light fading, heat fading, print out and yellowing in the manner described and the results reported in Table I (infra).

16 (B) Three film test strips are prepared and tested as in A (supra) but with the same amount of 1-hydroxy-4-chloro-2 - N[ $\alpha$ -(2,4-di-tert.-amylphenoxy)butyl]naphthamide (i.e., the two-equivalent 4-chloro analog) as the coupler, and the test results reported in Table I.

17 (C) Three film test strips are prepared and tested as in A (supra) but with Coupler XV having the formula



35 (D) Three test strips are prepared and tested as in A, utilizing as coupler 2,5-di-lauroylamidophenol obtained from the corresponding 5-amino-2-lauroylamidophenol and lauroyl chloride in accordance with the process described in Example V, and the test results reported in Table I.

40 (E) Three test strips are prepared and tested as in A, utilizing Coupler XXXIII (the two-equivalent 4-phenyl sulfonamido derivative) and the test results reported in Table I.

45 (F) Three test strips are prepared and tested as in A, utilizing as a coupler, a compound of the formula



55 (G) Three test strips are prepared and tested as in A, utilizing as a coupler, a compound of the formula



65 Light fading tests

70 The extent to which the image dyes fade under the influence of light is determined by subjecting processed coatings to a simulated 21-day north skylight exposure (SANS) and determining the resulting decrease in dye density in an area having an initial dye density of approximately 1.2. The resulting "Light Fade" is recorded as density units. The extent to which unreacted coupler

causes unwanted stain under the influence of light is determined by exposing processed coatings to SANS, as above described, and recording the resulting increase in density to blue light (420 m $\mu$ ) in a D min area of the coating. This increase is termed "Printout" (PO) and is recorded in terms of percent density increase.

#### Heat fading tests

The extent to which the image dyes fade under the influence of heat and humidity is determined by subjecting coatings to a temperature of 60° C. at a relative humidity of 70% for 1 week. The resulting decrease in image dye density is termed "Heat Fade" (H.F.) and is measured in terms of decrease in dye density in density units. The effect of heat on unreacted coupler is determined by subjecting coatings to the above heat and humidity conditions, and determining the increase in density (i.e., yellowing) in a D min area (420 m $\mu$ ) of the coating, and recording this in terms of percent density increase.

TABLE I

| Group          | Light fade | Heat fade | Printout, percent | Yellow, percent |
|----------------|------------|-----------|-------------------|-----------------|
| A              | .17        | .12       | 12                | 5               |
| B              | .11        | .05       | 7                 | 3               |
| C <sup>1</sup> | .13        | .06       | 6                 | 0               |
| D              | .15        | .13       | 10                | 7               |
| E <sup>1</sup> | .12        | .04       | 5                 | 2               |
| F              | .07        | .10       | 8                 | 3               |
| G <sup>1</sup> | .04        | .07       | 5                 | 1               |

<sup>1</sup> Contains a coupler of the invention.

The invention has been described in detail with particular reference to preferred embodiments thereof, but it will be understood that variations and modifications may be effected within the spirit and scope of the invention as described hereinabove and as defined in the appended claims.

We claim:

1. A photographic silver halide emulsion containing a phenol or  $\alpha$ -naphthol photographic color coupler having substituted in the No. 4 position of the phenolic and  $\alpha$ -naphtholic ring a sulfonamido group wherein the amido moiety of the sulfonamido group is attached at said No. 4 position.

2. A photographic silver halide emulsion containing a cyan-dye-forming color coupler compound of the formula



wherein COUP— is the residue of a cyan dye-forming coupler moiety of the phenolic or  $\alpha$ -naphtholic type;  $\text{R}_1-\text{SO}_2-\text{NH}-$  represents a non-chromophoric radical attached onto the No. 4 carbon of the phenol or  $\alpha$ -naphthol ring of COUP—; and  $\text{R}_1$  is an alkyl or an aryl group.

3. A photographic silver halide emulsion or emulsion layer containing at least one cyan dye-forming color coupler compound of the formulae



or



wherein (PHOL) and (NAOL) are respectively defined as a cyan-dye-forming coupler moiety of the phenolic or the  $\alpha$ -naphtholic type, the



group being a No. 4 phenolic- or No. 4- $\alpha$ -naphtholic ring substituent, the  $\text{R}_1$  moiety alone or in combination with any other part of the No. 4 ring substituent group being a non-chromophoric group and defined as an alkyl or an aryl group;

$\text{R}_3$  is a No. 2 phenolic ring-substituent defined as a hydrogen atom, an alkyl group having up to 30 carbon atoms,



wherein A is an unsubstituted alkyl group having up to 5

to 30 carbon atoms, a halo alkyl, or an aryloxy alkylene group; Ar is defined as an aryl group having one or more of an alkyl, an alkoxy, or a halo substituent group thereon, the alkyl moiety of said alkyl or alkoxy groups containing at least 15 carbon atoms; and

$\text{R}_7$  is a No. 2  $\alpha$ -naphtholic ring substituent defined as an alkyl group having up to 30 carbon atoms,



4. A photographic silver halide emulsion or emulsion layer containing at least one cyan-dye-forming coupler compound of the formulae



or



wherein (PHOL) and (NAOL) are respectively defined as the residue of a four-equivalent cyan-dye-forming coupler moiety of the phenolic or  $\alpha$ -naphtholic type having at least two substituent groups in phenolic or  $\alpha$ -naphtholic ring in addition to a hydroxy radical, the  $\text{R}_1-\text{SO}_2-\text{NH}$ -group being a No. 4 phenolic- or No. 4  $\alpha$ -naphtholic-ring substituent, the  $\text{R}_1$  moiety alone or in combination with any other part of the No. 4 ring substituent being a non-chromophoric group and defined as a straight or branched chain alkyl having 1-20 carbon atoms, a phenyl group, or a naphthyl group;

$\text{R}_3$  is a No. 2 phenolic ring substituent defined as an alkyl group having at least 15 carbon atoms



in which A is an unsubstituted alkyl group containing at least 15 carbon atoms, a halo alkyl, or an aryloxy alkylene group wherein the alkylene moiety contains up to 15 carbon atoms;

Ar is a phenyl or a naphthyl group; and

$\text{R}_7$  is a No. 2  $\alpha$ -naphtholic ring substituent defined as an alkyl group having at least 15 carbon atoms,



5. A photographic silver halide emulsion or emulsion layer of claim 3 wherein  $-(\text{PHOL})$  and  $-(\text{NAOL})-$ , respectively, have the formulae



55 in which

$\text{R}_2$  is defined as a hydrogen atom, a halo radical, an alkyl group having 1-20 carbon atoms, or an alkoxy group having an alkyl moiety of 1-20 carbon atoms;

$\text{R}_4$  is defined as a hydrogen atom, a halo radical, an alkyl group, or an alkoxy group;

$\text{R}_5$  in Formula 9 is defined as  $\text{R}_4$  and in Formula 8 additionally includes a radical of the formula



in which Y is an alkanoic acid group, an arylcarbonyl group, or a heterocyclic carbonyl having 5-6 members in the ring nucleus; and  $\text{R}_6$  and  $\text{R}_8$  are individually defined as a hydrogen atom or an alkyl group.

6. A photographic silver halide emulsion of claim 4 wherein

$\text{R}_2$  is a hydrogen, a lower alkyl, a lower alkoxy, or a halo group;

$\text{R}_4$  is a hydrogen atom, a halo group, a lower alkyl group, or a lower alkoxy group;



21

veloping agent and a diffusible cyan dye-forming coupler compound of the formula



wherein  $R_1$  is a phenylsulfonamido, a naphthyl sulfonamido, or an alkyl sulfonamido group having 1-20 carbon atoms;

$R_2$  is a hydrogen atom, a halo radical, a lower alkyl group, or a lower alkoxy group;

$R_3$  and  $R_7$  are each a hydrogen atom, an alkyl group having up to 14 carbon atoms, an alkoxy group having up to 14 carbon atoms,

$-\text{NH}-\text{CO}-\text{A}$  or  $-\text{CO}-\text{NH}-\text{A}$

wherein  $A$  is an alkyl group having up to 14 carbon atoms;  $R_{4-6}$  are each a hydrogen atom, a halo radical, a lower alkyl group, or a lower alkoxy group.

22. A color photographic developer composition comprising a p-phenylene-diamine color developing agent and a diffusible cyan dye-forming phenolic or  $\alpha$ -naphtholic type coupler selected from the group consisting of

2,6-dimethyl-4-phenylsulfonamidophenol,  
4-(m-nitrophenylsulfonamido)-phenol,  
4-( $\alpha$ -naphthyl sulfonamido)phenol,  
2-methyl-4-(phenylsulfonamido)phenol,  
3-methyl-6-isopropyl-4-phenylsulfonamidophenol,  
2,6-dimethyl-4-methylsulfonamidophenol,  
4-(phenylsulfonamido) $\alpha$ -naphthol,  
2-methyl-4-(phenylsulfonamido)- $\alpha$ -naphthol,  
4-( $\alpha$ -naphthylsulfonamido)- $\alpha$ -naphthol,  
2-methoxy-4-phenylsulfonamidophenol,  
4-phenylsulfonamidophenol,  
5-methoxy-5-phenylsulfonamidophenol,  
4-(p-nitrophenylsulfonamido)phenol, and  
2-(n-buty carbamyl)-4-phenylsulfonamidophenol.

23. A color photographic developer composition of claim 22 wherein the cyan dye-forming coupler is



24. A color photographic developer composition of claim 22 wherein the cyan dye-forming coupler is



5

22

25. A color photographic developer composition of claim 22 wherein the cyan dye-forming coupler is



10

26. A color photographic developer composition of claim 22 wherein the cyan dye-forming coupler is



15

27. A color photographic developer composition of claim 22 wherein the cyan dye-forming coupler is



30

35

28. The process for color developing an imagewise exposed photographic element comprising a support having coated thereon a photographic silver halide emulsion containing a phenol or  $\alpha$ -naphthol photographic color coupler having substituted in the No. 4 position of the phenolic and  $\alpha$ -naphtholic ring a sulfonamido group wherein the amido moiety of the sulfonamido group is attached to said No. 4 position, which process comprises developing said photographic element with an aqueous alkaline solution containing an aromatic primary amino color developing agent, and resulting oxidized color developing agent reacting in areas of silver halide development with said No. 4 position of said phenolic or  $\alpha$ -naphtholic ring to form a dye with said ring.

#### References Cited

#### UNITED STATES PATENTS

55 2,356,475 8/1944 Schinzel \_\_\_\_\_ 96-56.6  
2,362,598 11/1944 Vittum et al. \_\_\_\_\_ 96-56.6

NORMAN G. TORCHIN, Primary Examiner

60 R. L. SCHILLING, Assistant Examiner

U.S. CL. X.R.

96-100